

## UNITED STATES PATENT OFFICE

2,507,244

SURGICAL GELATIN DUSTING POWDER AND  
PROCESS FOR PREPARING SAMEJohn T. Correll, Kalamazoo, Mich., assignor to  
The Upjohn Company, Kalamazoo, Mich., a  
corporation of MichiganNo Drawing. Application April 14, 1947,  
Serial No. 741,419

5 Claims. (Cl. 260—117)

1

This invention relates to a powder, suitable for surgical use, which is absorbable by the bodies of living animals.

The technique of surgery, as developed through years of experience, requires the surgeon, after having thoroughly disinfected his hands, to wear rubber gloves during the actual manipulative performance. These rubber or surgical gloves are of a special construction, which is necessary according to the nature of their use. To allow snug fitting of the hand, the gloves must be extremely thin. This thinness, however, is disadvantageous in that it renders the gloves weak from a mechanical standpoint so that they are not capable of withstanding extensive pulling or stretching. To obviate tearing while they are in the process of being put on just before surgery, experience has shown that the gloves must be lubricated.

The most common lubricant for this use, until the present invention, has been a special sterile powdered inorganic talc. This talc, which is water-soluble and, by the nature of its physical structure, lubricating, allows the tight-fitting gloves to be fitted to the hand, and removed therefrom, without their rupture, and is therefore satisfactory for the surgeon's immediate purpose, viz, donning the gloves without their rupture or contamination. However, this talc is not entirely satisfactory from the standpoint of ultimate physiological effects upon the patient being treated.

It is well known that inert substances, foreign in composition to the body, exert a deleterious effect when allowed to remain in contact with the healing surfaces of an incision. This reaction, called a foreign-body reaction, instigates a permanent and progressive inflammation which may cause many complications, such as adhesions. Inert foreign bodies in the incision may also cause granulomatous lesions of the peritoneum, draining sinuses, scar nodules, and malfunctioning intestinal stoma.

It has been shown (Seelig, Verda, and Kidd, Jour. Am. Med. Assoc. 123, 950, 1943; Seelig, The Surgical Clinics of No. Am., Oct. 1944, Barnard Hospital Number; Seelig and Verda, Jour. Mount Sinai Hospital XII No. 1, May-June 1945; Seelig, Jour. So. Med. Assoc. 38, 470, 1945; Lichtman, McDonald, Dixon, and Mann, Surg. Gync. and Obst. 83, 531, 1946; Antopol, Arch. Path. 16, 326, 1933; Erb, Surg. Gyn. and Obst. 60, 40, 1935) that the talc commonly used in surgical procedures acts as a foreign body, with the above-mentioned undesirable results. The need for a lubricant which can be used in the same manner as talc, but

2

which does not have the attendant undesirable properties of talc, has been recognized in the references already given. These references further show that various attempts to solve this problem have been made, but no success is indicated.

It is, therefore, an object of the present invention to provide a powder which is suitable for use as a lubricant of such surgical devices as rubber gloves, but which, being absorbable by the body fluids, does not effect complications which arise from the employment of an inert material. As the new powder is water-insoluble, it is neither dissolved by perspiration nor made tacky or sticky by exposure thereto. The product of this invention is a water-insoluble, sterile, non-toxic, non-antigenic, non-tissue irritating hardened gelatin powder which is absorbable by the animal body without residue or untoward side reactions, and which is capable of safe and satisfactory lubrication of rubber articles such as the aforementioned surgical gloves.

The proteolytically digestible powder of the invention is prepared by suitably hardening a gelatin, either before or after reduction to a powder. 25 A gelatin solution may first be hardened either by the use of a chemical hardening agent, such as an aldehyde, or by heat, and thereafter subjected in either flake, slab, or powder form, to the synergistic action of a high-temperature treatment. Gelatin flake may be suitably hardened by merely heating the same, in its flake form or after further reduction to a powder, at a temperature above about 145 degrees centigrade for a period of time between about 20 and about 100 hours.

35 The degree to which the gelatin is changed or hardened is of critical importance, for, if the change from the original gelatin is not sufficient, the resulting product will be water-soluble or partially water-soluble and the powder will lose a certain proportion of its lubricating properties when exposed to moisture. On the other hand, if the change or hardening be carried too far, the product will no longer be susceptible to proteolytic disintegration and absorption by the body fluids, and thus, not being absorbable by the body, will cause the formation of granulomas and adhesions in the same manner as any other foreign substance. Accordingly, to determine whether the product has been suitably hardened, it should be found to be water-insoluble and proteolytically digestible. The digestion time may be determined in a manner similar to that employed for determining the proteolytic absorbability of cat gut sutures, such as, for example, by exposure

## 3

to either a 5.0 or 0.5 per cent pepsin solution, in which case proteolytic digestibility is usually satisfactory if complete within a period of about one-half hour and about six hours, respectively, for the two concentrations given. Beyond these limits, the product may be unsuited for the prescribed use.

The powder should not comprise any ingredients of an antigenic nature, but, while pure gelatin with or without a minor proportion of aldehydic hardening agent is presently considered the most satisfactory composition, other non-antigenic, sterile ingredients may be added, if such addition is considered desirable.

The hardening agent, if such is employed, may be of any suitable type, formaldehyde being preferred. This aldehydic hardening agent may be present in an amount not to exceed about three per cent by weight in the powdered product. Any other method of hardening a gelatin solution may be employed, provided only that the desired water-insoluble, non-antigenic, proteolytically-digestible powder be produced thereby. Circulation of air having a relative humidity of ten per cent or less at a temperature between about 20 and about 35 degrees centigrade, most desirably at about 30 degrees centigrade, is a satisfactory method of drying partially-solidified gelatin slabs, but spray-drying before gelation of the solution is complete may be employed if desired, and in some instances is preferred.

While the starting material for the preparation of the new gelatin powder may comprise either a gelatin solution or gelatin flake, and while the particular starting material may be dried and hardened in any suitable manner, the synergistic effect of drying at relatively higher temperatures as a step for the attainment of the proper physical properties is requisite. This step comprises subjecting the dry gelatin flake or powder to a relatively high temperature above about 145 degrees centigrade for a relatively lengthy period of time, e.g., from about 20 to 100 hours, preferably at a temperature between about 162 and 191 degrees centigrade (320 to 375 degrees Fahrenheit). This treatment has been found to produce the most suitably hardened or denatured gelatin powder, when used alone or in combination with other steps. A combination of the formaldehyde treatment and this heat denaturing is a very practical manner of producing the product of the present invention. The finely-divided gelatin powder, when desired to be used as a lubricant for rubber articles demanding sterility, should of course be sterilized, and such is usually accomplished by heating at elevated temperatures as illustrated in the examples.

The following examples are given to illustrate the preparation of the product of this invention, but are in no way to be construed as limiting.

## Example 1.

One kilogram of skin gelatin flake is dissolved in 10 liters of warm water to make a 10 per cent gelatin solution. The solution is cooled to about 40 degrees centigrade and 10 milliliters of U. S. P. 40 per cent formaldehyde solution is added with stirring. The solution is allowed to stand at room temperature until a stiff gel forms, whereafter the jelly is cut into slabs of suitable size, preferably less than one inch thick, and dried by circulation of air of 10 per cent or less relative humidity at a temperature of about 30 degrees centigrade. The dried hardened gelatin flakes are then ground to a fine powder, which is heated

## 4

at a temperature of about 145 degrees centigrade for between 15 and 95 hours. This powder is finely pulverized and bolted to the desired particle size, less than 50 microns in diameter. After packaging in a suitable container, the powder is sterilized by heating in dry air at 145 degrees centigrade for four hours. The powdered product is biologically absorbable and causes no foreign body reaction in surgical use.

## Example 2

The procedure of Example 1 was substantially repeated except that the gelatin solution was spray-dried before gelation of the solution, instead of being dried by circulation of air and subsequently ground.

## Example 3

Skin gelatin flake was reduced to a powder, spread in thin layers on trays, and heated evenly throughout at a temperature of 145 degrees centigrade for a period of 20 to 95 hours. The powder was then further pulverized and bolted to the desired size, preferably 50 microns or less in diameter, and packaged in suitable containers and sterilized, e.g., by heating in dry air to a temperature of 145 degrees centigrade for a period of about four hours. The powder is suitably biologically absorbable and non-irritating to incised human tissue.

Various modifications may be made in the invention without departing from the spirit or scope thereof, and it is to be understood that I limit myself only as defined in the appended claims.

I claim:

1. A sterile, substantially water-insoluble, non-antigenic, completely proteolytically digestible powder suitable for surgical lubrication consisting essentially of gelatin that has been hardened to the stage of substantial water-insolubility and that has thereafter been pulverized and subjected to heat treatment, which powdered material is completely digestible within approximately 0.5 hour in a 5 percent and within approximately 6 hours in a 0.5 percent aqueous pepsin solution.

2. A sterile, substantially water-insoluble, non-antigenic, completely proteolytically digestible powder suitable for surgical lubrication consisting essentially of gelatin that has been hardened by treatment with less than approximately 3 percent by weight of formaldehyde in aqueous solution, thereafter dried and pulverized and subjected to heat treatment until the product is no longer substantially soluble in water but still is completely digestible within approximately 0.5 hour in a 5 percent and within approximately 6 hours in a 0.5 percent aqueous solution of pepsin.

3. A sterile powder suitable for surgical lubrication as defined in claim 2 and further characterized in that the individual particles thereof are of a size less than approximately 50 microns in diameter.

4. A process for the production of a substantially water-insoluble, non-antigenic, completely proteolytically digestible powder suitable for surgical lubrication, which comprises: hardening gelatin to a state of substantial water-insolubility and thereafter heating said product at a temperature between approximately 145 degrees and approximately 191 degrees centigrade for such period that the product is substantially water-insoluble but still is completely proteolytically digestible.

5. A process for the production of a substantially water-insoluble, non-antigenic, completely

proteolytically digestible powder suitable for surgical lubrication, which comprises: treating an aqueous solution of gelatin with formaldehyde in an amount less than approximately 3 percent by weight of the gelatin until the gelatin is hardened to a state of substantial water-insolubility, thereafter drying said product at a temperature below approximately 35 degrees centigrade, pulverizing the dried product and heating the pulverized product at a temperature between approximately 145 degrees and approximately 191 degrees centigrade for such period that the product is substantially water-insoluble but still is completely proteolytically digestible.

JOHN T. CORRELL. 15

## REFERENCES CITED

The following references are of record in the file of this patent:

## UNITED STATES PATENTS

| Number       | Name     | Date          |
|--------------|----------|---------------|
| 658,747      | Altschul | Oct. 2, 1900  |
| 659,204      | Brat     | Oct. 9, 1900  |
| 10 1,021,674 | Horowitz | Mar. 26, 1912 |

## FOREIGN PATENTS

| Number  | Country | Date          |
|---------|---------|---------------|
| 555,718 | Germany | July 27, 1932 |

**Certificate of Correction**

Patent No. 2,507,244

May 9, 1950

**JOHN T. CORRELL**

It is hereby certified that error appears in the printed specification of the above numbered patent requiring correction as follows:

Column 1, line 22, for the hyphenated word "water-soluble" read *water-insoluble*; and that the said Letters Patent should be read as corrected above, so that the same may conform to the record of the case in the Patent Office.

Signed and sealed this 3rd day of October, A. D. 1950.

[SEAL]

**THOMAS F. MURPHY,**  
*Assistant Commissioner of Patents.*